

July 26, 1938.

S. P. MILLER

2,124,860

REFINING PROCESS

Filed March 11, 1936

Fig. 1.



Fig. 2.



INVENTOR

Stuart P. Miller

BY  
John Libby  
ATTORNEY

## UNITED STATES PATENT OFFICE

2,124,860

## REFINING PROCESS

Stuart Parmelee Miller, Scarsdale, N. Y., assignor  
to The Barrett Company, New York, N. Y., a  
corporation of New Jersey

Application March 11, 1936, Serial No. 68,229

4 Claims. (Cl. 75—65)

This invention relates to the refining of metals, and more particularly, to the melting and refining of non-ferrous metals in a cupola furnace.

This invention is in the nature of an improvement on the invention of the Cushion Reissue Patent No. 17,347, of July 2, 1929. That patent discloses a method of refining non-ferrous metals in a cupola furnace involving the placing of a charge of non-ferrous metal on a bed of pitch coke and burning the coke in contact with the metal to supply the heat necessary to melt the metal. As pointed out in this patent, pitch coke is substantially free of ash, sulphur and other materials having a deleterious effect upon the 15 non-ferrous metals refined in the cupola. Hence, by following the practice of this patent, the non-ferrous metals withdrawn from the cupola are not contaminated by impurities contained in the fuel employed in the cupola but are in a refined state 20 of high quality and do not require a subsequent refining operation.

By the term "non-ferrous metal" as used in the specification and claims herein are meant those metals other than ferrous metals which can be 25 practically melted in a cupola furnace and this term is intended to include the metals lead, copper, nickel, aluminum, tin, antimony, zinc, and alloys thereof but to exclude easily oxidizable metals such as magnesium, and alkali and alkali 30 earth metals.

It is an object of this invention to provide a process for melting and refining metals, and particularly non-ferrous metals, which minimizes the amount of fuel consumed in the cupola in contact with the metal being melted. Another object 35 is to provide a process of melting metals, and particularly non-ferrous metals, which is simple and economical to practice and which results in the production of a highly refined metal.

In accordance with this invention, the major, 40 if not the entire, amount of heat necessary to melt the metals in the cupola is produced by burning, externally of the cupola, fuel, such as pulverized or liquid pitch, pitch coke, petroleum coke, tar, 45 petroleum oil such as is used in oil-fired metallurgical furnaces, or gas, which fuels are substantially free of ash and materials having a deleterious effect upon the metal. Preferably, but not necessarily, an excess of oxygen-containing 50 gas, such as air, is employed to support combustion of the fuel. The heating gases thus produced are introduced and passed through a bed on which the charge of metal to be melted is supported in the cupola. This bed is preferably a 55 bed of relatively low-ash and low-sulfur coke,

such as pitch coke or petroleum coke, the use of such materials minimizing the amount of slag formed and the amount of deleterious impurities taken up by the molten metal.

In cases where excess oxygen-containing gas is 5 employed to support combustion of the fuel, the excess oxygen in the heating gases supports combustion of a portion of the coke bed, resulting in higher temperatures in the cupola than would be possible if such combustion did not take place. 10 The heating gases augmented by the products of combustion of the coke in the cupola then pass over the metal charge, heating the same to melting temperatures. The amount of oxygen introduced into the cupola with the heating gases is 15 controlled so that combustion of a relatively small proportion only of the charge of coke in the cupola takes place and the gases leaving the charge of coke and contacting with the metal contain little if any free oxygen. Hence, as a 20 neutral or reducing atmosphere is maintained in the metal-containing zone of the cupola, excessive oxidation of the metal is avoided.

By producing the heating gases necessary to melt the metal externally of the cupola and passing the same through the charge in the cupola, as contrasted with prior practice involving the blowing of air under pressure through the charge, it is possible to avoid an excessive oxidizing atmosphere in the cupola and so avoid metal losses 25 occurring when an excessive oxidizing atmosphere is maintained in the metal-containing zone of the cupola to support combustion of coke therein. Furthermore, the use of fuels substantially free of ash, sulphur and other material deleterious to 30 the metal, to produce the heating gases which are passed through the metal, results in a substantially pure refined metal since the combustion gases do not introduce troublesome impurities 35 into the metal. The highest quality of metal is 40 further insured by the employment of pitch or petroleum coke to support the charge of metal in the cupola. Pitch and petroleum cokes are sufficiently free of ash and other deleterious impurities 45 so that substantially no slag beyond that arising from impurities in the metals charged is formed in the cupola; this simplifies the melting and refining process by minimizing opportunity for the production of impurities in and their introduction 50 into the refined metal. As hereinabove indicated, the introduction of heating gases containing free oxygen, results in a partial combustion of the coke supporting the metal producing a high temperature in the cupola so that the maxi- 55

mum refining effect on the metal undergoing treatment is obtained.

In the accompanying drawing forming a part of the specification and showing for purposes of exemplification a preferred form of apparatus for practicing this invention without limiting the claimed invention to such illustrative instance, Fig. 1 is a side elevation, partly in section of such apparatus, and Fig. 2 is a plan view of the apparatus of Fig. 1.

Referring to the drawing, reference numeral 1 indicates a cupola furnace which may be of any well known type employed in the melting of metals. As shown in the drawing, the cupola 15 may comprise a suitable cylindrical shell 2 lined with refractory material 3 surmounted by a stack 4 and having a charging inlet 5 situated in the upper part of the shell and a tap opening 6 at the bottom. As needed, sand bed 7 may be disposed at the base of the cupola with its face inclined downwardly toward the tap opening 6.

In accordance with this invention, gas distributing bustle pipe 8 is disposed concentrically about the cupola, near the base portion thereof. 25 The bustle pipe 8 communicates with the interior portion of the cupola by means of conduits or tuyères 9, four such conduits being shown in Fig. 2. Conduit 10 connects the bustle pipe with combustion chamber 11 lined with refractory material 12. A fuel burner 13 extends through the rear wall 14 of the combustion chamber and communicates with a mixing chamber 15 provided with an air or other oxygen-containing gas inlet line 16 and a line 17 for supplying liquid or 30 gaseous fuel, such as liquid tar, pitch, petroleum oil, etc. The air entering 16 may be preheated by passage in heat exchange relation with the combustion chamber or otherwise before introduction into the mixing chamber. In case it is 35 desired to employ solid fuel substantially free of sulphur and of other materials deleterious to the metal being refined, such, for example, as pulverized pitch coke, a hopper 18 may be placed in communication with the mixing chamber by means of a valve controlled line 19 substantially as shown. Coarse coke may be burned on grates in a Dutch oven, in a shaft furnace, etc. and the 40 hot gaseous products of combustion free from deleterious impurities introduced into the cupola.

In the preferred operation of my invention a 50 charge of coke substantially free of ash, sulphur and other materials deleterious to the metal being refined, such as, for instance, petroleum coke or pitch coke is placed on the sand bed. It is 55 especially advantageous to employ pitch coke made in a beehive oven such as described in the aforementioned Cushing patent. The metalliferous charge which may be impure copper, bronze or other metals is then placed upon the bed of coke. If liquid or gaseous fuel free of sulphur, ash and other constituents deleterious to the metal being refined is employed, as for example, liquid tar, pitch, petroleum, or combustible gas, such fuel is admitted into the mixing chamber 15 through line 17. Air or other oxygen-containing gas introduced through line 60 16 mixes with the fuel, and the mixture passes to the burner 13 where it is ignited by the high temperature prevailing in the combustion chamber. Preferably, an excess amount of air is introduced into the mixing chamber such that the gases entering the coke charge contain from 65 five to fifteen per cent. free oxygen. This free oxygen supports combustion of a portion of the coke. In melting non-ferrous metals, e. g. 70

bronze, by the process of the above mentioned Cushing patent, a ratio of metal melted to fuel consumed of from 10 to 18 parts by weight of metal to 1 part of fuel is ordinarily obtained, although under some conditions a ratio as high 5 as 20:1 may be reached. In accordance with the present invention the ratio of metal melted to bed fuel in the cupola consumed is greatly increased; for example, a ratio greater than 20:1 is usually obtained and this ratio may even be 10 40:1 or higher depending on combustion conditions in the burner and fuel bed as above described. The waste hot gas leaves through stack 4, and the molten metal is withdrawn through tap hole 6.

In cases where an excess of oxygen-containing gas is not employed to support combustion of the fuel burned externally of the cupola, air or other oxygen-containing gas may be introduced into the cupola in amount sufficient to support combustion 20 of a portion of the pitch or other coke supporting the metal charge.

If solid fuel is utilized to supply the heat necessary to melt the charge, fuel reservoir 18 is supplied with pulverized pitch or other finely 25 divided combustible material which is substantially free from ash, sulphur and other materials deleterious to the metal being refined. Air is admitted through inlet 16 at a pressure which may be of the order of 2 to 5 pounds per square 30 inch, into the mixer where it mixes with the solid fuel. The resulting fuel mix passes to the combustion chamber through burner 13 where it is ignited and burns with the resultant formation of hot gases. The hot gases are led through 35 the bustle pipe 8, through conduits 9 into the interior of the cupola, through the coke bed and into contact with the metallic charge, thereby melting it. The molten metal trickles through the hot coke bed and is removed through tap 40 opening 6. Alternatively solid fuel may be burned on a grate or in other suitable apparatus outside the cupola, and the hot combustion gases introduced into the cupola through pipe 10. Since such combustion apparatus is well known, 45 it is not illustrated in the drawing.

It will be noted that in accordance with this invention the cost of melting metal is substantially reduced as compared with the use of coke, particularly pitch coke, as the fuel, since only a 50 portion of such coke is consumed, the major portion of the heat being supplied by the burning of relatively low cost fuels externally of the cupola. Further, the temperature in the melting zone can be accurately controlled when operating in accordance with this invention by regulation of combustion in the muffle furnace or combustion chamber 11. If desired, the muffle furnace lining may be built up from air-cooled bricks, the air passing through the bricks being introduced 60 into the mixing chamber to support combustion of the fuel buried externally of the cupola or introduced directly into the cupola to support combustion of the pitch coke or other coke employed to support the metal charge. Melting conditions 65 may further be regulated by choice of fuels. Fuels giving highly luminous flames, e. g., tar, pitch, may be used to give high speed melting whereas fuels, such as natural gas, resulting in relatively non-luminous flames, may give relatively low speed melting.

While as hereinabove pointed out, the bed of fuel for supporting the molten metal within the cupola is preferably a bed of low-ash and low-sulphur coke, such as pitch or petroleum coke, in 75

many cases it is not necessary to use a bed of such high purity as pitch or petroleum coke, since in my process a relatively small ratio of coke to metal melted is consumed in the cupola. 5 In fact, ordinary furnace or foundry coke (made from coal) will be satisfactory for some purposes. Practically all of the impurities taken up by molten metal in the process of the present invention are taken up from the coke bed and slag with 10 which the metal is in contact. When, as in the present process, the major portion of the heat for melting is supplied by combustion of fuel outside of the cupola, the combustion of coke inside the cupola is reduced to a small fraction of the usual 15 amount and hence opportunity for absorption of impurities by the metal from the coke bed and slag is correspondingly reduced. Under such conditions, ordinary foundry coke may be of sufficient purity for use as the bed in the cupola. 20

Since certain changes may be made in carrying out the above process without departing from the scope of the invention, it is intended that all matter contained in the above description shall 25 be interpreted as illustrative and not in a limiting sense. For example, while a bed of pitch or petroleum coke has been disclosed as the support for the metal charge, and such bed is preferred and should be employed to obtain all the 30 benefits of this invention, a bed of other coke (as above pointed out), such as ordinary coke, either high or low temperature coke, charcoal, or of refractory material capable of supporting the burden, may be employed in lieu of pitch coke and 35 the metal charge which may be bronze, lead, dross, copper, cast iron or steel heated by passing the products of combustion free of deleterious constituents thereover.

What is claimed is:

40 1. In the operation of a cupola furnace for the melting of non-ferrous metal, those steps which comprise placing a bed of coke substantially free of ash and other materials having a deleterious effect upon the non-ferrous metal within the cupola, placing a charge of non-ferrous metal 45 on said bed of coke, producing heating gases by the combustion of fuel substantially free of ash and other material having a deleterious effect upon said non-ferrous metal, said heating gases 50 containing a controlled excess of free oxygen, passing said heating gases into said furnace and in controlled amount into contact with said coke, the excess of free oxygen therein consuming a controlled minor portion only of said coke bed in 55 the cupola so as to avoid an excessive oxidizing atmosphere in the cupola and thereby avoiding excessive metal losses from said charge, passing the resultant heating gases through said charge of non-ferrous metals to heat the metals to melting temperatures, and withdrawing the molten 60 metal from the cupola.

2. The method of refining non-ferrous metals in a cupola furnace in which the non-ferrous metal is supported on a charge of pitch coke substantially free of ash and material having a deleterious effect upon the non-ferrous metal, which comprises producing, externally of the cupola, heating gases by the combustion of fuel substantially free of ash and of material having a deleterious effect upon the non-ferrous metal, utilizing a controlled excess of oxygen-containing gas 5 to support combustion of said fuel, passing the heating gases through the pitch coke and the non-ferrous metal to be refined in the cupola, the excess of free oxygen supporting combustion of 10 the pitch coke within the cupola, the amount of free oxygen in the heating gases being controlled so that only a minor portion of the charge of pitch coke within the cupola is consumed in the melting of the non-ferrous metal. 15

3. The method of refining non-ferrous metals in a cupola furnace in which the non-ferrous metal is supported on a charge of pitch coke substantially free of ash and of materials having a deleterious effect upon the non-ferrous metal, which comprises producing, externally of the 20 cupola, heating gases by the combustion of liquid fuel substantially free of ash and materials having a deleterious effect upon the non-ferrous metal, utilizing a controlled excess of oxygen-containing gas to support the combustion of said fuel, passing the heating gases through the pitch coke, the amount of free oxygen in the heating gases being controlled so that only a controlled minor portion of the supporting charge of coke 25 is consumed, and passing the heating gases augmented by products of combustion of the pitch coke over the non-ferrous metal to melt the same. 30

4. In the operation of a cupola furnace for the melting of non-ferrous metal, those steps which comprise placing a charge of coke substantially free of ash and other materials having a deleterious effect upon the non-ferrous metal within the cupola, placing a charge of non-ferrous metal on said charge of coke, producing heating gases by the combustion of fuel substantially free of ash and other material having a deleterious effect upon said non-ferrous metal, said heating gases 45 containing an excess of free oxygen, passing said heating gases into said furnace and into contact with said coke, the excess of free oxygen therein supporting combustion of a portion of the coke within the cupola, passing the resultant heating gases through said charge of non-ferrous metals to heat the metals to melting temperatures, and withdrawing the molten metal from 50 the cupola, the ratio of metal melted to coke consumed being greater than 20:1. 55

60 STUART PARMELEE MILLER.